

J. P. WATERS.

HIGH SPEED STEEL AND PROCESS OF FORMING AND FORGING THE SAME.

APPLICATION FILED AUG. 16, 1916.

1,345,045.

Patented June 29, 1920.

Fig. 1.



Fig. 2.



Fig. 3.



Fig. 4.



Fig. 5.

Inventor  
James P. Waters

By *Whittenton, Hubert & Whittenton*

Attorneys

# UNITED STATES PATENT OFFICE.

JAMES P. WATERS, OF DETROIT, MICHIGAN, ASSIGNOR, BY MESNE ASSIGNMENTS, TO FORGE PRODUCTS CORPORATION, OF ANN ARBOR, MICHIGAN, A CORPORATION OF NEW YORK.

## HIGH-SPEED STEEL AND PROCESS OF FORMING AND FORGING THE SAME.

1,345,045.

Specification of Letters Patent. Patented June 29, 1920.

Application filed August 16, 1916. Serial No. 115,221.

To all whom it may concern:

Be it known that I, JAMES P. WATERS, a citizen of the United States of America, residing at Detroit, in the county of Wayne and State of Michigan, have invented certain new and useful Improvements in High-Speed Steel and Processes of Forming and Forging the Same, of which the following is a specification, reference being had thereto in the accompanying drawings.

The invention relates to the manufacture of tools and other articles from what is known in the art as high speed steel, meaning by this term metal having tungsten, vanadium and chromium, or other ingredients having similar properties. The better qualities of high speed steel may contain up to say, 17% to 19% tungsten; 3½% to 4½% chromium; ½% to 1½% of the vanadium; and say ½% to ¾% of carbon. In the present state of the art steels of this character are usually heat treated at temperatures above 2000° F., both in the original forging of the stock from ingots and in the subsequent tempering. The metal at this temperature is not, however, capable of being worked or fashioned in the same manner as an ordinary carbon steel, and all attempts at drop forging or otherwise re-forging the metal have resulted in failure. This is for the reason that the metal is lacking in density and at the temperature described it will inevitably fracture under the operation of a die or drop hammer.

I have discovered that high speed steels may be successfully forged by limiting the temperature to 2000° F. or under, and I have further discovered that metal fashioned in this manner is improved in quality, having greater homogeneity, density and tensile strength. Still another advantage is that the metal so fashioned may be successfully tempered within a greater range of temperature variation than has been heretofore possible.

My invention is applicable to the manufacture of any articles from high speed steel, but I shall specifically describe the process of forming a milling cutter, as shown in the accompanying drawings, in which Figure 1 is an elevation of a cut-off section of stock before the forging operation; Figs. 2 and 3 are respectively a plan view and a side elevation after the preliminary

blanking operation; Fig. 4 is a side elevation of the refashioned blank; and Fig. 5 is a plan view indicating in dotted lines the manner in which the blank may be sheared or trimmed.

The stock from which the article is to be formed is preferably cut off to the proper size or weight, as shown in Fig. 1. The severed section is then heated to the temperature of approximately 1900° F. and is refashioned by hammering, pressing or other mechanical means, as shown in Figs. 2 and 3. After this blanking operation the metal is again re-heated, preferably to a temperature of approximately 1800° F. and is fashioned to its final form as shown in Fig. 4, by drop forging or otherwise. If the cutting-off of the blank from the stock is by a hot process, the temperature should be less than 2000° F., preferably about 1900° F.

As a result of the several operations and successive heating and working of the metal, it is changed in its physical character, becoming more homogeneous and of increased density and tensile strength. The essential feature of the process is the limiting of the temperature to less than 2000° F., preferably about 1900° F. and, as specifically described, the final re-fashioning is at still lower temperature, say 1800° F. Of course, the precise temperatures named can never be exactly obtained in practice and some variations are permissible to suit different conditions and qualities of the steel.

Tools or other articles which are fashioned in the manner described are greatly improved in strength and durability, and furthermore are more easily tempered, which operation may be successfully performed within a range of temperature variation from 2100° F. to 2300° F. for the quenching heat, and from 380° F. to 1100° for the drawing heat, these limits being more extended than has heretofore been feasible.

After the final re-fashioning operation, the metal is preferably annealed, and if desired annealing steps may be introduced intermediate the several steps in the process.

As shown in Figs. 1 to 3, the blanking operation is preferably performed by upsetting the stock so as to spread the metal transversely of the grain thereof. This endwise upsetting and transverse working of the

metal is an important feature of the invention and I have discovered that blanks made in this way possess great strength, density and homogeneity.

- 5 5. What I claim as my invention is:—
  1. The process of fashioning articles from high speed steel, comprising the forging or working of the metal at a temperature of less than 2000° F. to form a rough blank,
  - 10 10. and the subsequent re-fashioning of the blank at a lesser temperature.
  - 15 2. The process of forming articles from high speed steel, comprising the forging or working of the metal at a temperature no higher than 2000° F. to form a rough blank, 15 re-forging the blank at a lower temperature, and finally annealing.
  - 20 3. The process of forming articles from high speed steel, comprising the heating of the stock to a temperature of less than 2000° F. and severing a section therefrom, re-heating the severed section to a temperature of less than 2000° F. and forging the same into a rough blank, and re-heating the blank to
  - 25 25. a temperature of less than 1900° F. and forging the same to its final form.
  - 30 4. In a process of forming articles from high speed steel, the step of upsetting or transversely working the metal at a temperature of less than 2000° F.
  - 35 5. The process of fashioning articles from high speed steel, comprising the upsetting or transverse working of the metal at a temperature of less than 2000° F. to form a rough blank, and the subsequent re-fashioning of the blank in dies at a lower temperature.
  - 40 6. The process of forming articles from high speed steel, comprising the cutting of the blank from stock of lesser diameter than the finished article, heating and upsetting said blank to diminish the length and increase the diameter thereof and thereby to

increase the density and homogeneity of the metal, and re-fashioning in dies to the desired form.

7. As a new product, an upset or transversely-worked blank of high-speed steel having the characteristics of increased density and greater homogeneity, as compared to a blank of the same material, otherwise produced.

8. The process of forging high speed tungsten steel of the class described, which process comprises severing from the stock a blank of the proper volume but of dimensions different from those of the finished article, refashioning and spreading the material of the blank toward the desired dimensions by hot forging at approximately 1900° F. and further refashioning the blank by a reheating and another forging operation starting with a temperature substantially less than 1900° F.

9. The process of forming articles from high speed steel stock of the class described, which method comprises severing from the stock a blank of dimensions substantially differing from those of the finished article, refashioning and spreading the material of the blank toward the desired dimensions by a hot forging operation, starting with a temperature of approximately 1900° F. and further refashioning the blank by a reheating and another forging operation starting with a temperature of approximately 1800° F.

10. The process of forming articles from high speed steel of the class described, which consists in performing successive operations on the metal at successive heats each beginning at approximately 1900° F. followed by another heating and metal fashioning operation starting at a substantially lower temperature.

In testimony whereof I affix my signature. 85  
JAMES P. WATERS.